

# United States Patent [19]

Pollastrini et al.

[11] Patent Number: 4,956,324

[45] Date of Patent: Sep. 11, 1990

[54] CATALYST CONTAINING DIPOLAR COMPOUNDS USEFUL FOR SWEETENING A SOUR HYDROCARBON FRACTION

[75] Inventors: Sheila Pollastrini, Bloomingdale; Jeffery C. Bricker, Buffalo Grove; Robert R. Frame, Glenview, all of Ill.

[73] Assignee: UOP, Des Plaines, Ill.

[21] Appl. No.: 473,512

[22] Filed: Feb. 1, 1990

## Related U.S. Application Data

[63] Continuation-in-part of Ser. No. 386,923, Jul. 31, 1989.

[51] Int. Cl.<sup>5</sup> B01J 31/22

[52] U.S. Cl. 502/163; 502/164; 208/189; 208/203; 208/207

[58] Field of Search 502/163, 164; 208/189, 208/203, 207

## [56] References Cited

### U.S. PATENT DOCUMENTS

3,108,948 10/1963 Ring 208/189

|           |         |                |         |
|-----------|---------|----------------|---------|
| 4,298,463 | 11/1981 | Frame          | 208/189 |
| 4,498,977 | 2/1985  | Frame          | 208/207 |
| 4,498,978 | 2/1985  | Frame          | 208/207 |
| 4,502,949 | 3/1985  | Frame          | 208/207 |
| 4,672,047 | 6/1987  | Chandler       | 502/62  |
| 4,824,818 | 4/1989  | Bricker et al. | 502/163 |

Primary Examiner—Helane Myers

Attorney, Agent, or Firm—Thomas K. McBride; Eugene I. Snyder; Frank S. Molinaro

[57]

## ABSTRACT

This invention relates to an improved catalyst for treating a sour hydrocarbon stream. The improvement comprises the use of a dipolar compound which has a positively charged atom and an electronegative group in the same structure. A particularly preferred dipolar compound is ephedrine. The dipolar compounds may be used in conjunction with a metal chelate and a basic solution either in a liquid-liquid process or a fixed bed process with substantially increased performance for oxidizing mercaptans which are found in the sour hydrocarbon stream.

18 Claims, No Drawings

CATALYST CONTAINING DIPOLAR  
COMPOUNDS USEFUL FOR SWEETENING A  
SOUR HYDROCARBON FRACTION

CROSS REFERENCE TO RELATED  
APPLICATION

This application is a continuation-in-part of our co-pending application, Ser. No. 07/386,923 filed July 31, 1989, now U.S. Pat. No. 4,929,340.

BACKGROUND OF THE INVENTION

Processes for the treatment of a sour hydrocarbon fraction where the fraction is treated by contacting it with an oxidation catalyst and an alkaline agent in the presence of an oxidizing agent at reaction conditions have become well known and widely practiced in the petroleum refining industry. These processes are typically designed to effect the oxidation of offensive mercaptans contained in a sour hydrocarbon fraction to innocuous disulfides—a process commonly referred to as sweetening. The oxidizing agent is most often air. Gasoline, including natural, straight run and cracked gasolines, is the most frequently treated sour hydrocarbon fraction. Other sour hydrocarbon fractions which can be treated include the normally gaseous petroleum fraction as well as naphtha, kerosene, jet fuel, fuel oil, and the like.

A commonly used continuous process for treating sour hydrocarbon fractions entails contacting the fraction with a metal phthalocyanine catalyst dispersed in an aqueous caustic solution to yield a doctor sweet product. The sour fraction and the catalyst containing aqueous caustic solution provide a liquid-liquid system wherein mercaptans are converted to disulfides at the interface of the immiscible solutions in the presence of an oxidizing agent—usually air. Sour hydrocarbon fractions containing more difficult to oxidize mercaptans are more effectively treated in contact with a metal chelate catalyst dispersed on a high surface area adsorptive support—usually a metal phthalocyanine on an activated charcoal. The fraction is treated by contacting it with the supported metal chelate catalyst at oxidation conditions in the presence of an alkaline agent. One such process is described in U.S. Pat. No. 2,988,500. The oxidizing agent is most often air admixed with the fraction to be treated, and the alkaline agent is most often an aqueous caustic solution charged continuously to the process or intermittently as required to maintain the catalyst in the causticwetted state.

The prior art shows that the usual practice of catalytically treating a sour hydrocarbon fraction containing mercaptans involves the introduction of alkaline agents, usually sodium hydroxide, into the sour hydrocarbon fraction prior to or during the treating operation. See U.S. Pat. Nos. 3,108,081 and 4,156,641. The prior art also discloses that quaternary ammonium compounds can improve the activity of these catalytic systems. For example, see U.S. Pat. Nos. 4,290,913 and 4,337,147. In these patents the catalytic composite comprises a metal chelate, an alkali metal hydroxide and a quaternary ammonium hydroxide dispersed on an adsorptive support.

The prior art also discloses the use of other nitrogen-containing compounds as promoters for mercaptan sweetening. For example, U.S. Pat. No. 4,207,173 discloses the use of guanidine as a promoter for mercaptan oxidation. Further, U.S. Pat. No. 4,753,722 discloses a

large number of nitrogen-containing compounds as promoters. These compounds are classified as heterocyclic compounds, substituted homocyclic compounds and aliphatic compounds.

In contrast to this prior art, applicants have found that a dipolar compound can greatly promote the oxidation of mercaptans in both liquid-liquid and fixed bed processes. A dipolar compound is an organic compound which has a positively charged atom and an electronegative group in the same structure.

The dipolar compounds of this invention can have the structural formula



25 where Z is nitrogen or phosphorus, R, R<sub>1</sub>, R<sub>2</sub>, R<sub>3</sub>, and R<sub>4</sub> are groups as defined herein and X is halogen or hydroxide.

A preferred class of dipolar compounds are betaines which have the general formula



35 where R' is an alkyl, alkaryl, aralkyl and cycloalkyl group. An especially preferred dipolar compound is ephedrine which has the formula



45 and in which the hydroxyl group is capable of being deprotonated. There is no mention in the prior art that such dipolar compounds would be effective promoters for the oxidation of mercaptans. Further, applicants have found that the dipolar compounds are much more active promoters than quaternary ammonium compounds.

50 It is noted that these dipolar compounds superficially appear to resemble quaternary ammonium compounds (when Z is nitrogen), especially structure (A). However, there are several differences between these dipolar compounds and quaternary ammonium salts. First, the electronegative group on the dipolar compound is covalently attached to the remainder of the compound, i.e., it is a functional group, whereas the quaternary salt has a positive ion and a negative ion which are held in close proximity by ionic forces. Therefore, the negative ion in the quaternary salt can be removed and exchanged with a resin or other chemical means. An example of this type of exchange is shown by the following equation:



55 In contrast to this, the electronegative group on the dipolar compound cannot be exchanged with a resin or

chemical means. The only way to remove the electronegative group is to break a covalent bond.

Second, the association between negative and positive ions in a salt are different from that found between the negative and positive groups in the dipolar compound. The dipolar compound may have the positive and negative groups physically separated and acting independently, whereas in a quaternary salt the counter ion must be in close proximity to balance the positive charge.

Third, the counter ions of the quaternary salts are relatively inert in catalysis reactions, whereas the electronegative groups present on the dipolar compounds can be catalytically active. That is, it makes very little difference whether the counter ion is chloride, hydroxide, acetate, etc., whereas changing the electronegative group from OH to COOH or SO<sub>3</sub>H can effect the properties of the dipolar compound.

However, even if the dipolar compounds were considered to be structurally equivalent to a quaternary salt, the prior art does not provide any hint or motivation to add an electronegative group as a functional group to any of the groups attached to the nitrogen atom. Further, there is no indication in the prior art that a quaternary ammonium compound containing an electronegative group would be a better promoter than a quaternary ammonium compound without an electronegative group. Applicants are the first to have discovered this unexpected result.

#### SUMMARY OF THE INVENTION

It is a broad objective of this invention to present improved processes and catalysts for treating a sour hydrocarbon fraction containing mercaptans. Thus, one broad embodiment of the invention is a process for treating a sour hydrocarbon fraction containing mercaptans comprising contacting the hydrocarbon fraction in the presence of an oxidizing agent with a basic solution containing a metal chelate effective in oxidizing said mercaptans to disulfides, wherein the improvement comprises a dipolar compound present in the basic solution, the dipolar compound having the structural formula



where Z is nitrogen or phosphorus, R is a linear group having from one to about 18 carbon atoms, R<sub>1</sub> and R<sub>2</sub> are each individually hydrogen or a hydrocarbon group selected from the group consisting of alkyl, aryl, alkaryl, aralkyl and cycloalkyl, R<sub>3</sub> and R<sub>4</sub> are each individually a hydrocarbon group selected from the group consisting of alkyl, aryl, alkaryl, aralkyl and cycloalkyl, YH is an electronegative group selected from the group consisting of OH, SH, COOH, SO<sub>3</sub>H and NH<sub>2</sub>, the electronegative group characterized in that it is capable of being deprotonated in a basic solution, and X is an anion selected from the group consisting of the halogens and hydroxide; or the structural formula



where Y<sup>-</sup> is the deprotonated form of YH.

Another embodiment of the invention is a process for treating a sour hydrocarbon fraction containing mercaptans comprising contacting the hydrocarbon fraction in the presence of an oxidizing agent with a basic solution containing a metal chelate effective in oxidizing said mercaptans to disulfides, wherein the improvement comprises a dipolar compound present in the basic solution, the dipolar compound selected from the group consisting of an ephedrine compound, an ephedrine salt and mixtures thereof, where the ephedrine compound has the structural formula



where R<sub>5</sub> is hydrogen or an alkyl group having from 1 to about 25 carbon atoms and the ephedrine salt has the structural formula



where R<sub>5</sub> is as defined above, R<sub>6</sub> is an alkyl or cycloalkyl group having from 1 to about 25 carbon atoms and X is an anion selected from the group consisting of hydroxide, chloride and bromide.

Yet another embodiment of the invention is a process for treating a sour hydrocarbon fraction containing mercaptans comprising contacting the hydrocarbon fraction in the presence of an oxidizing agent and a basic agent with a catalyst effective in oxidizing the mercaptans to disulfides, wherein the improvement comprises a catalyst comprising an adsorbent support having dispersed thereon a metal chelate and a dipolar compound having the structural formula



where Z is nitrogen or phosphorus, R is a linear alkyl group having from one to about 18 carbon atoms, R<sub>1</sub> and R<sub>2</sub> are each individually hydrogen or a hydrocarbon group selected from the group consisting of alkyl, aryl, alkaryl, aralkyl and cycloalkyl, R<sub>3</sub> and R<sub>4</sub> are each individually a hydrocarbon group selected from the group consisting of alkyl, aryl, alkaryl, aralkyl and cycloalkyl, YH is an electronegative group selected from the group consisting of OH, SH, COOH, SO<sub>3</sub>H and NH<sub>2</sub>, the electronegative group characterized in that it is capable of being deprotonated in a basic solution, and X is an anion selected from the group consisting of the halogens and hydroxide; or the structural formula



(B)

5

where  $\text{Y}^-$  is the deprotonated form of  $\text{YH}$ .

Still another embodiment of the invention is a process for treating a sour hydrocarbon fraction containing mercaptans comprising contacting the hydrocarbon fraction in the presence of an oxidizing agent and a basic agent with a catalyst effective in oxidizing the mercaptans to disulfides, wherein the improvement comprises a catalyst comprising an adsorbent support having dispersed thereon a metal chelate and a dipolar compound selected from the group consisting of an ephedrine compound, an ephedrine salt or a mixture thereof as described above.

A further broad embodiment of the invention is a catalyst effective for oxidizing mercaptans present in a sour hydrocarbon fraction comprising a basic solution containing a metal chelate and a promoter which is a dipolar compound having the structural formula



(A)

25

where  $\text{Z}$  is nitrogen or phosphorus,  $\text{R}$  is a linear alkyl group having from one to about 18 carbon atoms,  $\text{R}_1$  and  $\text{R}_2$  are each individually hydrogen or a hydrocarbon group selected from the group consisting of alkyl, aryl, alkaryl, aralkyl and cycloalkyl,  $\text{R}_3$  and  $\text{R}_4$  are each individually a hydrocarbon group selected from the group consisting of alkyl, aryl, alkaryl, aralkyl and cycloalkyl,  $\text{YH}$  is an electronegative group selected from the group consisting of  $\text{OH}$ ,  $\text{SH}$ ,  $\text{COOH}$ ,  $\text{SO}_3\text{H}$  and  $\text{NH}_2$ , the electronegative group characterized in that it is capable of being deprotonated in a basic solution, and  $\text{X}$  is an anion selected from the group consisting of the halogens and hydroxide; or the structural formula



(B)

35

where  $\text{Y}^-$  is the deprotonated form of  $\text{YH}$ .

Still another embodiment of the invention is a catalyst effective for oxidizing mercaptans present in a sour hydrocarbon fraction comprising an adsorbent support having dispersed thereon a metal chelate and a dipolar compound having the structural formula



(A)

55

where  $\text{Z}$  is nitrogen or phosphorus,  $\text{R}$  is a linear alkyl group having from one to about 18 carbon atoms,  $\text{R}_1$  and  $\text{R}_2$  are each individually hydrogen or a hydrocarbon group selected from the group consisting of alkyl, aryl, alkaryl, aralkyl and cycloalkyl,  $\text{R}_3$  and  $\text{R}_4$  are each individually a hydrocarbon group selected from the group consisting of alkyl, aryl, alkaryl, aralkyl and cycloalkyl,  $\text{YH}$  is an electronegative group selected from the group consisting of  $\text{OH}$ ,  $\text{SH}$ ,  $\text{COOH}$ ,  $\text{SO}_3\text{H}$  and  $\text{NH}_2$ , the electronegative group characterized in that it is capable of being deprotonated in a basic solution, and  $\text{X}$  is an anion selected from the group consisting of the halogens and hydroxide; or the structural formula

$\text{NH}_2$ , the electronegative group characterized in that it is capable of being deprotonated in a basic solution, and  $\text{X}$  is an anion selected from the group consisting of the halogens and hydroxide; or the structural formula



(B)

where  $\text{Y}^-$  is the deprotonated form of  $\text{YH}$ .

A further embodiment of the invention is a catalyst effective for oxidizing mercaptans present in a sour hydrocarbon fraction comprising an adsorbent support having dispersed thereon a metal chelate and a dipolar compound selected from the group consisting of an ephedrine compound, an ephedrine salt and mixtures thereof as described above.

Yet another embodiment of the invention is a catalyst effective for oxidizing mercaptans in a sour hydrocarbon fraction comprising a basic solution containing a metal chelate and a dipolar compound selected from the group consisting of an ephedrine compound, an ephedrine salt and mixtures thereof as described above.

Other objects and embodiments of this invention will become apparent in the following detailed description of the invention.

#### DETAILED DESCRIPTION OF THE INVENTION

As stated, this invention relates to improved processes and catalysts for treating a sour hydrocarbon fraction. The process comprises contacting a sour hydrocarbon fraction in the presence of an oxidizing agent with a catalyst. The catalyst can be present either in a liquid phase (liquid-liquid sweetening) or as a solid phase (fixed bed sweetening).

The liquid-liquid process comprises contacting the sour hydrocarbon fraction with a basic solution containing a metal chelate and a dipolar compound. The basic solution is an aqueous solution containing from about 0.1 to about 25 weight percent, preferably from about 0.1 to about 10 weight percent, and most preferably from about 0.5 to about 7 weight percent of an alkali metal hydroxide or ammonium hydroxide. Of the alkali metal hydroxides, sodium and potassium hydroxides are preferred, although lithium hydroxide, rubidium hydroxide and cesium hydroxide may also be used. The metal chelate employed in the practice of this invention can be any of the various metal chelates known to the art as effective in catalyzing the oxidation of mercaptans contained in a sour petroleum distillate, to disulfides or polysulfides. The metal chelates include the metal compounds of tetrapyrnidinoporphyrazine described in U.S. Pat. No. 3,980,582, e.g., cobalt tetrapyrnidinoporphyrazine; porphyrin and metaloporphyrin catalysts as described in U.S. Pat. No. 2,966,453, e.g., cobalt tetraphenylporphyrin sulfonate; corrinoid catalysts as described in U.S. Pat. No. 3,252,892, e.g., cobalt corrin sulfonate; chelate organometallic catalysts such as described in U.S. Pat. No. 2,918,426, e.g., the condensation product of an aminophenol and a metal of Group VIII; the metal phthalocyanines as described in U.S. Pat. No. 4,290,913, etc. As stated in U.S. Pat. No. 4,290,913, metal phthalocyanines are a preferred class of metal chelates. All the above-named patents are incorporated herein by reference.

The metal phthalocyanines which can be employed in the basic solution to catalyze the oxidation of mercaptans generally include magnesium phthalocyanine, titanium phthalocyanine, hafnium phthalocyanine, vanadium phthalocyanine, tantalum, phthalocyanine, molybdenum phthalocyanine, manganese phthalocyanine, iron phthalocyanine, cobalt phthalocyanine, platinum phthalocyanine, palladium phthalocyanine, copper phthalocyanine, silver phthalocyanine, zinc phthalocyanine, tin phthalocyanine, and the like. Cobalt phthalocyanine and vanadium phthalocyanine are particularly preferred. The ring substituted metal phthalocyanines are generally employed in preference to the unsubstituted metal phthalocyanine (see U.S. Pat. No. 4,290,913), with the sulfonated metal phthalocyanine being especially preferred, e.g., cobalt phthalocyanine monosulfate, cobalt phthalocyanine disulfonate, etc. The sulfonated derivatives may be prepared, for example, by reacting cobalt, vanadium or other metal phthalocyanine with fuming sulfuric acid. While the sulfonated derivatives are preferred, it is understood that other derivatives, particularly the carboxylated derivatives, may be employed. The carboxylated derivatives are readily prepared by the action of trichloroacetic acid on the metal phthalocyanine. The concentration of metal chelate in general and metal phthalocyanine in specific in the basic solution can vary from about 0.1 to about 2000 ppm and preferably from about 50 to about 800 ppm.

The dipolar compound which may be used as a promoter along with the metal chelate in the basic solution has the formula



where Z is nitrogen or phosphorus, R is a linear alkyl group having from one to about 18 carbon atoms, R<sub>1</sub> and R<sub>2</sub> are each individually hydrogen or a hydrocarbon group selected from the group consisting of alkyl, aryl, alkaryl, aralkyl and cycloalkyl, R<sub>3</sub> and R<sub>4</sub> are each individually a hydrocarbon group selected from the group consisting of alkyl, aryl, alkaryl, aralkyl and cycloalkyl, YH is an electronegative group selected from the group consisting of OH, SH, COOH, SO<sub>3</sub>H and NH<sub>2</sub>, the electronegative group characterized in that it is capable of being deprotonated in a basic solution, and X is an anion selected from the group consisting of the halogens and hydroxides; or the structural formula



where Y<sup>-</sup> is the deprotonated form of YH. Specifically, the deprotonated forms of the YH groups enumerated above are O<sup>-</sup>, S<sup>-</sup>, COO<sup>-</sup>, SO<sub>3</sub><sup>-</sup>, and NH<sup>-</sup>. A preferred counter ion, X, is chloride. It should be pointed out that regardless of which structure the dipolar compound has, when it is dissolved in a basic solution the dipolar compound exists to at least some measurable extent as structure (B) or what is usually referred to as an inner salt or a zwitter ion. The choice of using the dipolar compound in form A or B is merely a choice of convenience and availability and does not affect the

activity of the dipolar compound. Illustrative examples of the dipolar compounds which can be used to practice this invention, but which are not intended to limit the scope of this invention are Z=nitrogen, Y<sup>-</sup>=COO<sup>-</sup>, R<sub>1</sub>=H, R=CH<sub>2</sub>, R<sub>2</sub>=R<sub>3</sub>=R<sub>4</sub>=ethyl; Z=nitrogen, Y<sup>-</sup>=COO<sup>-</sup>, R<sub>1</sub>=H, R=CH<sub>2</sub>, R<sub>2</sub>=R<sub>3</sub>=R<sub>4</sub>=methyl; Z=nitrogen, Y<sup>-</sup>=COO<sup>-</sup>, R<sub>1</sub>=H, R=CH<sub>2</sub>, R<sub>2</sub>=hexadecyl, R<sub>3</sub>=R<sub>4</sub>=methyl; Z=nitrogen, Y<sup>-</sup>=COO<sup>-</sup>, R<sub>1</sub>=H, R=(CH<sub>2</sub>)<sub>3</sub>, R<sub>2</sub>=R<sub>3</sub>=R<sub>4</sub>=methyl; Z=nitrogen, Y<sup>-</sup>=COO<sup>-</sup>, R<sub>1</sub>=H, R=(CH<sub>2</sub>)<sub>3</sub>, R<sub>2</sub>=decyl, R<sub>3</sub>=R<sub>4</sub>=methyl; Z=nitrogen, Y<sup>-</sup>=COO<sup>-</sup>, R<sub>1</sub>=H, R=(CH<sub>2</sub>)<sub>6</sub>, R<sub>2</sub>=R<sub>3</sub>=R<sub>4</sub>=methyl; Z=nitrogen, Y<sup>-</sup>=COO<sup>-</sup>, R<sub>1</sub>=H, R=CH<sub>2</sub>, R<sub>2</sub>=coco, R<sub>3</sub>=R<sub>4</sub>=methyl; Z=nitrogen, Y<sup>-</sup>=COO<sup>-</sup>, R<sub>1</sub>=H, R=CH<sub>2</sub>, R<sub>2</sub>=tallow, R<sub>3</sub>=R<sub>4</sub>=methyl; Z=nitrogen, YH=SO<sub>3</sub>H, R<sub>1</sub>=H, R=(CH<sub>2</sub>)<sub>2</sub>, R<sub>2</sub>=tallow, R<sub>3</sub>=R<sub>4</sub>=methyl, X=Cl; Z=nitrogen, YH=SO<sub>3</sub>H, R<sub>1</sub>=H, R=tallow, R<sub>2</sub>=R<sub>3</sub>=R<sub>4</sub>=methyl, X=Cl; Z=nitrogen, YH=COOH, R<sub>1</sub>=H, R=CH<sub>2</sub>, R<sub>2</sub>=tallow, R<sub>3</sub>=R<sub>4</sub>=methyl, X=Cl; Z=nitrogen, YH=OH, R<sub>1</sub>=H, R=(CH<sub>2</sub>)<sub>4</sub>, R<sub>2</sub>=decyl, R<sub>3</sub>=R<sub>4</sub>=methyl, X=Cl; Z=phosphorus, Y<sup>-</sup>=COO<sup>-</sup>, R<sub>1</sub>=H, R=CH<sub>2</sub>, R<sub>2</sub>=R<sub>3</sub>=R<sub>4</sub>=methyl; Z=phosphorus, Y<sup>-</sup>=COO<sup>-</sup>, R<sub>1</sub>=H, R=CH<sub>2</sub>, R<sub>2</sub>=decyl, R<sub>3</sub>=R<sub>4</sub>=methyl; Z=phosphorus, Y<sup>-</sup>=COO<sup>-</sup>, R<sub>1</sub>=H, R=decyl, R<sub>2</sub>=R<sub>3</sub>=R<sub>4</sub>=methyl; Z=phosphorus, YH=COOH, R<sub>1</sub>=H, R=(CH<sub>2</sub>)<sub>3</sub>, R<sub>2</sub>=R<sub>3</sub>=R<sub>4</sub>=methyl, X=Cl; Z=phosphorus, YH=COOH, R<sub>1</sub>=H, R=CH<sub>2</sub>, R<sub>2</sub>=coco, R<sub>3</sub>=R<sub>4</sub>=methyl, X=Cl.

15

20

25

30

35

40

45

50

55

60

65

60

65

70

75

80

85

90

95

100

105

110

115

120

125

130

135

140

145

150

155

160

165

170

175

180

185

190

195

200

205

210

215

220

225

230

235

240

245

250

255

260

265

270

275

280

285

290

295

300

305

310

315

320

325

330

335

340

345

350

355

360

365

370

375

380

385

390

395

400

405

410

415

420

425

430

435

440

445

450

455

460

465

470

475

480

485

490

495

500

505

510

515

520

525

530

535

540

545

550

555

560

565

570

575

580

585

590

595

600

605

610

615

620

625

630

635

640

645

650

655

660

665

670

675

680

685

690

695

700

705

710

715

720

725

730

735

740

745

750

755

760

765

770

775

780

785

790

795

800

805

810

815

820

825

830

835

840

845

850

855

860

865

870

875

880

885

890

895

900

905

910

915

920

925

930

935

940

945

950

955

960

965

970

975

980

985

990

995

1000

1005

1010

1015

1020

1025

1030

1035

1040

1045

1050

1055

1060

1065

1070

1075

1080

1085

1090

1095

1100

1105

1110

1115

1120

1125

1130

1135

dodecyl, etc. The ephedrine salts have the structural formula



where R<sub>5</sub> is hydrogen or an alkyl group having from 1 to about 25 carbon atoms, R<sub>6</sub> is an alkyl, alkaryl or cycloalkyl group having from 1 to about 25 carbon atoms and X is an anion selected from the group consisting of hydroxide, chloride, bromide, iodide and fluoride. Ephedrine is an especially preferred dipolar compound. Mixtures of the ephedrine compounds and ephedrine salts may be used in the practice of the invention.

Regardless of the dipolar compound actually used, it is desirable that the dipolar compound be present in the basic solution in a concentration from about 0.1 to about 400 ppm, preferably from about 1 to about 100 ppm and most preferably from about 3 to about 20 ppm.

Sweetening of the sour hydrocarbon fraction is effected by oxidation of mercaptans. Accordingly, an oxidizing agent is necessary for the reaction to proceed. Air is a preferred oxidizing agent, although oxygen or other oxygen-containing gases may be used. At least a stoichiometric amount of oxygen (relative to the concentration of mercaptans) is required to oxidize the mercaptans to disulfides, although an excess amount of oxygen is usually employed. In some cases the sour hydrocarbon fraction may contain entrained air or oxygen in sufficient concentration to accomplish the desired sweetening, but generally it is preferred to introduce air into the reaction zone.

Sweetening of the sour hydrocarbon fraction may be effected in any suitable manner well known in the art and may be in a batch or continuous process. In a batch process the sour hydrocarbon fraction is introduced into a reaction zone containing the basic solution which contains the metal chelate and the dipolar compound. Air is introduced therein or passed therethrough. Preferably the reaction zone is equipped with suitable stirrers or other mixing devices to obtain intimate mixing. In a continuous process the basic solution containing the metal chelate catalyst and the dipolar compounds is passed countercurrently or concurrently with the sour hydrocarbon fraction in the presence of a continuous stream of air. In a mixed type process, the reaction zone contains the basic solution, metal chelate and dipolar compound, and gasoline and air are continuously passed therethrough and removed generally from the upper portion of the reaction zone. For specific examples of apparatus used to carry out a liquid/liquid process, see U.S. Pat. Nos. 4,019,869, 4,201,626 and 4,234,544 which are incorporated by reference.

In general the process is usually effected at ambient temperatures, although elevated temperatures may be employed and generally will be in the range of from about 100° to about 400° F., depending upon the pressure utilized therein, but usually below that at which substantial vaporization occurs. Pressures of up to about 1,000 psi or more are operable although atmospheric or substantially atmospheric pressures are suitable.

The process may also be carried out by contacting the sour hydrocarbon fraction with a catalyst comprising a metal chelate and a dipolar compound dispersed on an adsorbent support. This is referred to as fixed bed

sweetening. The adsorbent support which may be used in the practice of this invention can be any of the well known adsorbent materials generally utilized as a catalyst support or carrier material. Preferred adsorbent materials include the various charcoals produced by the destructive distillation of wood, peat, lignite, nutshells, bones, and other carbonaceous matter, and preferably such charcoals as have been heat-treated or chemically treated or both, to form a highly porous particle structure of increased adsorbent capacity, and generally defined as activated carbon or charcoal. Said adsorbent materials also include the naturally occurring clays and silicates, e.g., diatomaceous earth, fuller's earth, kieselguhr, attapulgus clay, feldspar, montmorillonite, halloysite, kaolin, and the like and also the naturally occurring or synthetically prepared refractory inorganic oxides such as alumina, silica, zirconia, thoria, boria, etc., or combinations thereof like silica-alumina, silica-zirconia, alumina-zirconia, etc. The adsorbent support should be insoluble in, and otherwise inert to, the petroleum distillate at the alkaline reaction conditions existing in the treating zone. Charcoal, and particularly activated charcoal, is preferred because of its capacity for metal chelates, and because of its stability under treating conditions.

The metal chelates which can be deposited on the support are the ones that have been described above for the liquid-liquid process. Likewise, the dipolar compounds are the same as described above including ephedrine compounds and ephedrine salts.

The metal chelate component and dipolar compound can be dispersed on the adsorbent support in any conventional or otherwise convenient manner. The components can be dispersed on the support simultaneously from a common aqueous or alcoholic solution and/or dispersion thereof or separately and in any desired sequence. The dispersion process can be effected utilizing conventional techniques whereby the support in the form of spheres, pills, pellets, granules or other particles of uniform or irregular size or shape, is soaked, suspended, dipped one or more times, or otherwise immersed in an aqueous or alcoholic solution and/or dispersion to disperse a given quantity of the dipolar compound and metal chelate components. Typically, the dipolar compound will be present in a concentration of about 0.01 to about 5 weight percent of the catalyst and preferably from about 0.1 to about 3 weight percent. In general, the amount of metal chelate and metal phthalocyanine in particular which can be adsorbed on the solid adsorbent support and still form a stable catalyst is up to about 25 weight percent of the catalyst. A lesser amount in the range of from about 0.1 to about 10 weight percent of the catalyst generally forms a suitably active catalyst.

One preferred method of preparation involves the use of a steam-jacketed rotary dryer. The adsorbent support is immersed in the impregnating solution and/or dispersion containing the desired components contained in the dryer and the support is tumbled therein by the rotating motion of the dryer. Evaporation of the solution in contact with the tumbling support is expedited by applying steam to the dryer jacket. In any case, the resulting composite is allowed to dry under ambient temperature conditions, or dried at an elevated temperature in an oven, or in a flow of hot gases, or in any other suitable manner to yield a suitable catalyst.

An alternative and convenient method for dispersing the dipolar compound and metal chelate components on the solid adsorbent support comprises predisposing the support in a sour hydrocarbon fraction treating zone or chamber as a fixed bed and passing a metal chelate and dipolar compound solution and/or dispersion through the bed in order to form the catalytic composite in situ. This method allows the solution and/or dispersion to be recycled one or more times to achieve a desired concentration of the dipolar compound and metal chelate components on the adsorbent support. In still another alternative method, the adsorbent support may be predisposed in said treating zone or chamber, and the zone or chamber thereafter filled with the solution and/or dispersion to soak the support for a predetermined period.

Processes for sweetening a sour hydrocarbon fraction using a fixed bed catalyst are described in the prior art. Specifically, temperature and pressure conditions are the same as stated for the liquid-liquid process described above. The prior art also discloses (see U.S. Pat. Nos. 4,033,860 and 4,337,147) that the hydrocarbon fraction can be treated in the presence of a basic agent, usually an alkaline agent. Thus, a supported catalyst is typically initially saturated with an aqueous solution of an alkaline agent (as described above) and the alkaline agent thereafter passed in contact with the catalyst bed continuously or intermittently as required, admixed with the sour hydrocarbon fraction. An aqueous ammonium hydroxide solution (as described above) may be used in place of the alkaline solution. The aqueous solution may further contain a solubilizer to promote mercaptan solubility, e.g., alcohol, and especially methanol, ethanol, n-propanol, isopropanol, etc., and also phenols, cresols, and the like. The solubilizer, when employed, is preferably methanol, and the alkaline solution may suitably contain from about 2 to about 10 volume percent thereof. Examples of specific arrangements to carry out the treating process may be found in U.S. Pat. Nos. 4,490,246 and 4,753,722 which are incorporated by reference.

The following examples are presented in illustration of this invention and are not intended as undue limitations on the generally broad scope of the invention as set out in the appended claims.

#### EXAMPLE 1

A stirred contactor which consisted of a cylindrical glass container measuring 3.5 inches in diameter by 6 inches high and which contained 4 baffles that are at 90° angles to the side walls was used. An air driven motor was used to power a paddle stirrer positioned in the center of the apparatus. When turning, the stirrer paddles passed within  $\frac{1}{2}$ " of the baffles. This resulted in a very efficient, pure type of mixing.

To the above apparatus there were added 50 milliliters of an 8% aqueous sodium hydroxide solution which contained 30 weight ppm of a caustic soluble tetrasulfonated cobalt phthalocyanine and 200 milliliters of isoctane which contained 1,300 weight ppm of mercaptan sulfur as n-octylmercaptan. To this mixture 20 ppm of a mixture of quaternary ammonium compounds composed of alkyldimethylbenzyl ammonium chloride and dialkylmethylbenzyl ammonium chloride obtained from the Mason Chemical Co. as Maquat TC-76, was added and the mixture was stirred. Periodically stirring was stopped and a sample was withdrawn from the isoctane layer with a pipette. These samples were

analyzed for mercaptan by titration and are presented in Table 1.

#### EXAMPLE 2

The test described in Example 1 was carried out with a fresh sample of isoctane, cobalt phthalocyanine and alkaline solution, but instead of the quaternary ammonium compound, 20 ppm of ephedrine was added. These results are also presented in Table 1.

#### EXAMPLE 3

The test described in Example 1 was carried out with a fresh sample of isoctane, cobalt phthalocyanine and alkaline solution, but instead of the quaternary ammonium compound, 20 ppm of a betaine having the structural formula



obtained from Aldrich Chemical Co. was added. These results are also presented in Table 1.

TABLE 1

| Contact Time<br>(Minutes) | Effect of Dipolar Compounds on Mercaptan Oxidation |           |         |
|---------------------------|----------------------------------------------------|-----------|---------|
|                           | Quat OH                                            | Ephedrine | Betaine |
| 30                        | 10                                                 | 37        | 67      |
|                           | 20                                                 | 95        | 100     |
|                           | 30                                                 | 100       | 100     |
|                           | 50                                                 | 100       | 100     |
|                           | 70                                                 | 100       | 100     |
|                           | 90                                                 | 100       | 100     |

35 The data clearly show the superior promotion effect of dipolar compounds such as ephedrine and betaine.

We claim as our invention:

1. A catalyst effective for oxidizing mercaptans present in a sour hydrocarbon fraction comprising a basic solution containing a metal chelate and a promoter which is a dipolar compound having the structural formula



50 where Z is nitrogen or phosphorus, R is a linear alkyl group having from one to about 18 carbon atoms, R<sub>1</sub> and R<sub>2</sub> are each individually hydrogen or a hydrocarbon group selected from the group consisting of alkyl, aryl, alkaryl, aralkyl and cycloalkyl, R<sub>3</sub> and R<sub>4</sub> are each 55 individually a hydrocarbon group selected from the group consisting of alkyl, aryl, alkaryl, aralkyl and cycloalkyl, YH is an electronegative group selected from the group consisting of OH, SH, COOH, SO<sub>3</sub> H and NH<sub>2</sub>, the electronegative group characterized in that it is capable of being deprotonated in a basic solution, and X is an anion selected from the group consisting of the halogens and hydroxide; or the structural formula



where  $Y^-$  is the deprotonated form of  $YH$ .

2. The catalyst of claim 1 where  $R_3$  and  $R_4$  are both a linear alkyl group containing from about 5 to about 20 carbon atoms.

3. The catalyst of claim 1 where the basic solution is a sodium hydroxide solution containing from about 0.1 to about 25 weight percent sodium hydroxide.

4. The catalyst of claim 1 where the basic solution is an aqueous solution containing from about 0.1 to about 25 weight percent ammonium hydroxide.

5. The catalyst of claim 1 where the metal chelate is a metal phthalocyanine.

6. The catalyst of claim 5 where the metal phthalocyanine is a cobalt phthalocyanine and is present in a concentration from about 0.1 to about 2000 ppm.

7. A catalyst effective for oxidizing mercaptans present in a sour hydrocarbon fraction comprising a basic solution containing a metal chelate and a dipolar compound selected from the group consisting of an ephedrine compound, an ephedrine salt and mixtures thereof, the ephedrine compound has the structural formula



where  $R_5$  is hydrogen or an alkyl group having from 1 to about 25 carbon atoms, and the ephedrine salt has the structural formula



where  $R_6$  is an alkyl, alkaryl or cycloalkyl group having from 1 to about 25 carbon atoms and  $X$  is an anion selected from the group consisting of hydroxide, chloride, bromide, iodide and fluoride.

8. The catalyst of claim 7 where the basic solution is a sodium hydroxide solution containing from about 0.1 to about 25 weight percent sodium hydroxide.

9. The catalyst of claim 7 where the basic solution is an aqueous solution containing from about 0.1 to about 25 weight percent ammonium hydroxide.

10. The catalyst of claim 7 where the metal chelate is a metal phthalocyanine.

11. The catalyst of claim 10 where the metal phthalocyanine is a cobalt phthalocyanine and is present in a concentration from about 0.1 to about 2000 ppm.

12. A catalyst effective for oxidizing mercaptans present in a sour hydrocarbon fraction comprising an adsorbent support having dispersed thereon a metal chelate and a dipolar compound having the structural formula



(A)

where  $Z$  is nitrogen or phosphorus,  $R$  is a linear alkyl group having from one to about 18 carbon atoms,  $R_1$  and  $R_2$  are each individually hydrogen or a hydrocarbon group selected from the group consisting of alkyl, aryl, alkaryl, aralkyl and cycloalkyl,  $R_3$  and  $R_4$  are each individually a hydrocarbon group selected from the group consisting of alkyl, aryl, alkaryl, aralkyl and cycloalkyl,  $YH$  is an electronegative group selected from the group consisting of  $OH$ ,  $SH$ ,  $COOH$ ,  $SO_3H$  and

10  $NH_2$ , the electronegative group characterized in that it is capable of being deprotonated in a basic solution, and  $X$  is an anion selected from the group consisting of the halogens and hydroxide; or the structural formula

15



(B)

20 where  $Y^-$  is the deprotonated form of  $YH$ .

13. The catalyst of claim 12 where  $R_3$  and  $R_4$  are both a linear alkyl group containing from about 5 to about 20 carbon atoms.

14. The catalyst of claim 12 where the metal chelate is a metal phthalocyanine.

15. The catalyst of claim 14 where the metal phthalocyanine is a cobalt phthalocyanine and is present in a concentration from about 0.1 to about 10 weight percent of the catalyst.

16. A catalyst effective for oxidizing mercaptans present in a sour hydrocarbon fraction comprising an adsorbent support having dispersed thereon a metal chelate and a dipolar compound selected from the group consisting of an ephedrine compound, an ephedrine salt and mixtures thereof, the ephedrine compound has the structural formula



where  $R_5$  is hydrogen or an alkyl group having from 1 to about 25 carbon atoms, and the ephedrine salt has the structural formula



where  $R_6$  is an alkyl, alkaryl or cycloalkyl group having from 1 to about 25 carbon atoms and  $X$  is an anion selected from the group consisting of hydroxide, chloride, bromide, iodide and fluoride.

17. The catalyst of claim 16 where the metal chelate is a metal phthalocyanine.

18. The catalyst of claim 17 where the metal phthalocyanine is a cobalt phthalocyanine and is present in a concentration from about 0.1 to about 10 weight percent of the catalyst.

\* \* \* \* \*